

# United States Patent Office

2,719,101

Patented Sept. 27, 1955

1

2,719,101

## PRINTING OF TEXTILE PIECES

Adolf Koebner, Davyhulme, Urmston, England, assignor to Lankro Chemicals Ltd., Manchester, England, a corporation of Great Britain

No Drawing. Application November 24, 1951,  
Serial No. 258,099

Claims priority, application Great Britain  
December 27, 1950

9 Claims. (Cl. 154—149)

This invention relates to improvements in or relating to the printing of textiles.

In screen printing the pieces to be printed are spread out full-length on long tables and fastened to the table surface. This fastening can be done in different ways. The oldest method, which is still in use, consists in covering the table first with a felt and then with a piece of cotton (backgrey) and then fixing the goods to be printed with pins. Alternatively the pieces and backgrey are stuck together on a separate machine by using a water-soluble gum and the combined pieces are then fastened to the table by the aid of hooks provided on the two long sides of the table.

The method, however, most commonly used today is as follows:

The tables are covered with a water-repellent material such as leathercloth or rubber-faced cotton. A solution of gum arabic, dextrin or other natural gum is evenly distributed over the table; the piece is then rolled on and pressed against the table surface by a heavy roller. This method is a substantial improvement over the original method described hereinbefore, but it has a number of disadvantages including the following:

1. It is necessary to wash the table after each piece is printed and to renew the adhesive film. Color which has penetrated the piece sticks firmly to the table surface and the washing, therefore, takes a considerable length of time. On the other hand, any color accidentally left on the table surface will soil the subsequent piece.

2. As both pasting gum and printing color are usually water-soluble, there will be a tendency for the piece to come off the table on the printed parts.

3. Some of the pasting gum adheres to the back of the piece and hinders penetration of the printing color. The amount of gum on the back of the piece will not be the same all over the piece and, as it influences the shade obtained, there is always the danger of getting variations in shade, especially if big motives (blotches) are printed.

4. Color which penetrates the piece will combine with the gum on the table. It is, therefore, very difficult to get "through prints," i. e., equal printing results on the face and back of the piece.

5. It is not easy to remove the last traces of the pasting gum from the piece. These remnants of gums give the piece a harsh feel.

It is the principal object of the present invention to provide an improved textile printing process which overcomes the aforesaid disadvantages of the prior art practices.

Other objects, features and advantages of this invention will be apparent from the more detailed description which follows.

The present invention provides a method of printing textile pieces supported upon the surface of a table, such as in screen printing, wherein the pieces are removably affixed to the surface of the table by means of a tacky, water-repellent adhesive comprising a polymer of a higher aliphatic methacrylate derived from an aliphatic alcohol

2

containing from 6 to 12 carbon atoms or a copolymer of the said higher aliphatic methacrylate with a lower aliphatic acrylate or methacrylate derived from an aliphatic alcohol containing less than 6 carbon atoms.

5 The water-repellent adhesive can be applied to the surface of the table in solution in a volatile organic solvent, such as benzene, toluene, carbon tetrachloride or perchlorethylene, which evaporates after application. The solution may contain a second organic solvent or compatible substance which acts as an extender and/or plasticizer, for example cyclohexanol, cyclohexanone, butyl acetate, ethyl glycol acetate or butyl glycol or white spirits. White spirits or mineral spirits generally designate petroleum distillate serving as hydrocarbon solvents substantially all of which vaporizes between 160 and 200° C.

10 Alternatively the water-repellent adhesive can be applied in the form of an aqueous emulsion, which gives a continuous, tacky film on evaporation of the water.

15 20 The polymeric adhesive provides a permanently tacky surface, so that many pieces can be printed without renewing the adhesive film. As the film of adhesive is water-repellent, substantially no printing color sticks to the table and the washing of the table is greatly facilitated.

25 The printing color does not interfere with the water-repellent adhesive and no loosening of the adherence of the textile materials occurs during printing.

30 35 No traces of the adhesive can be found on the back of the piece and thus there is no danger of variation in shade.

As the water-repellent adhesive does not accept any printing color, all the color applied to the fabric is held by the printed material and perfect through-prints are obtained with a saving of color.

35 40 The feel or hand of the printed pieces is not affected by the method of this invention.

The following examples, in which the parts are expressed in parts by weight, constitute illustrative embodiments of the present invention.

### Example 1

45 One to 2 parts of benzoyl peroxide are added to a solution of 2-ethyl hexyl methacrylate (30 parts) in benzene (70 parts), and the mixture refluxed until the desired viscosity of the solution is obtained. The necessary refluxing requires 1 to 4 hours. Then 1 part of cyclohexanol is added to the solution. A coating of resultant solution is applied to the surface of a printing table and dries to a permanent, continuous, tacky, water-repellent film. A textile piece is affixed to the water-repellent film and screen-printed in the conventional manner.

### Example 2

50 55 n-Hexyl methacrylate is polymerized in a refluxing benzene solution, while adding gradually 5% by weight (calculated on the hexyl ester used) of methyl methacrylate. When the reaction mixture has obtained the desired viscosity the reaction is interrupted. The product is applied to the surface of a printing table and dries to a permanent, continuous, tacky, water-repellent film to which a textile piece is affixed and screen-printed in the conventional manner.

### Example 3

60 65 70 Thirty parts of 2-ethyl hexyl methacrylate monomer are emulsified in 70 parts of water by the addition of 1 part sodium lauryl sulphate, the mixture stirred at 70° C. and 1 part of ammonium persulphate added. Polymerization is complete after 3 hours. The resultant emulsion is applied to the surface of a printing table and dries to a permanent, continuous, tacky, water-repellent film to which a textile piece is affixed and screen-printed in the conventional manner.

The foregoing description constituting illustrative em-

bodiments of the invention is not to be considered a limitation upon the invention, for the invention contemplates various adaptations, alterations and modifications which would occur to those skilled in the art and would still be within the scope of the invention which is intended to be defined by the appended claims.

What is claimed is:

1. In the printing of textiles wherein the textile material is supported by being affixed to the surface of a table during printing, the improvement comprising bonding the textile material to the table with a permanently tacky, water-repellent polymer selected from the group consisting of a polymer of an ester of methacrylic acid with a high aliphatic alcohol containing 6 to 12 carbon atoms and copolymers of said ester with an ester of an acid selected from the group consisting of acrylic acid and methacrylic acid with a lower aliphatic alcohol containing less than 6 carbon atoms.

2. In the printing of textiles wherein the textile material is supported by being affixed to the surface of a table during printing, the improvement comprising applying to the surface of the table a coating containing an acrylic polymer selected from the group consisting of a polymer of an ester of methacrylic acid with a higher aliphatic alcohol containing 6 to 12 carbon atoms and copolymers of said ester with an ester of an acid selected from the group consisting of acrylic acid and methacrylic acid with a lower aliphatic alcohol containing less than 6 carbon atoms dispersed in a volatile organic solvent, and after the coating has dried to a permanently tacky, water-repellent film, affixing the textile material to the table through the bonding action of said dried coating.

3. In the printing of textiles wherein the textile material is supported by being affixed to the surface of a table during printing, the improvement comprising applying to the surface of the table a coating containing an acrylic polymer selected from the group consisting of a polymer of an ester of methacrylic acid with a higher aliphatic alcohol containing 6 to 12 carbon atoms and copolymers of said ester with an ester of an acid selected from the group consisting of acrylic acid and methacrylic acid with a lower aliphatic alcohol containing less than 6 carbon atoms dissolved in benzene, and after the coating has dried to a permanently tacky, water-repellent film, affixing the textile material to the table through the bonding action of said dried coating.

4. In the printing of textiles wherein the textile material is supported by being affixed to the surface of a table during printing, the improvement comprising applying to the surface of the table a coating containing an acrylic polymer selected from the group consisting of a polymer of an ester of methacrylic acid with a higher aliphatic alcohol containing 6 to 12 carbon atoms and copolymers of said ester with an ester of an acid selected from the group consisting of acrylic acid and methacrylic acid with a lower aliphatic alcohol containing less than 6 carbon atoms and an extender for the acrylic polymer dispersed in a volatile organic solvent, and after the coating has dried to a permanently tacky, water-repellent film, affixing the textile material to the table through the bonding action of said dried coating.

5. In the printing of textiles wherein the textile material is supported by being affixed to the surface of a table during printing, the improvement comprising applying to the surface of the table a coating containing an acrylic polymer selected from the group consisting of a polymer of an ester of methacrylic acid with a higher aliphatic al-

cohol containing 6 to 12 carbon atoms and copolymers of said ester with an ester of an acid selected from the group consisting of acrylic acid and methacrylic acid with a lower aliphatic alcohol containing less than 6 carbon atoms and cyclohexanol dissolved in benzene, and after the coating has dried to a permanently tacky, water-repellent film, affixing the textile material to the table through the bonding action of said dried coating.

6. In the printing of textiles wherein the textile material is supported by being affixed to the surface of a table during printing, the improvement comprising applying to the surface of the table a coating of an aqueous dispersion containing an acrylic polymer selected from the group consisting of a polymer of an ester of methacrylic acid with a higher aliphatic alcohol containing 6 to 12 carbon atoms and copolymers of said ester with an ester of an acid selected from the group consisting of acrylic acid and methacrylic acid with a lower aliphatic alcohol containing less than 6 carbon atoms, and after the coating has dried to a permanently tacky, water-repellent film, affixing the textile material to the table through the bonding action of said dried coating.

7. In the printing of textiles wherein the textile material is supported by being affixed to the surface of a table during printing, the improvement comprising bonding the textile material to the table with a permanently tacky, water-repellent polymer of 2-ethyl hexyl methacrylate.

8. In the printing of textiles wherein the textile material is supported by being affixed to the surface of a table during printing, the improvement comprising bonding the textile material to the table with a permanently tacky, water-repellent copolymer of n-hexyl methacrylate and methyl methacrylate.

9. In the printing of textiles wherein the textile material is supported by being affixed to the surface of a table during printing, the improvement comprising applying to the surface of the table a coating containing an acrylic polymer selected from the group consisting of a polymer of an ester of methacrylic acid with a higher aliphatic alcohol containing 6 to 12 carbon atoms and copolymers of said ester with an ester of an acid selected from the group consisting of acrylic acid and methacrylic acid with a lower aliphatic alcohol containing less than 6 carbon atoms dispersed in a hydrocarbon solvent having a boiling range between 160° and 200° C., and after the coating has dried to a permanently tacky, water-repellent film, affixing the textile material to the table through the bonding action of said dried coating.

#### References Cited in the file of this patent

#### UNITED STATES PATENTS

|           |                 |       |               |
|-----------|-----------------|-------|---------------|
| 1,982,946 | Bauer           | ----- | Dec. 4, 1934  |
| 2,098,118 | Wheelwright     | ----- | Nov. 2, 1937  |
| 2,217,133 | Overlack        | ----- | Oct. 8, 1940  |
| 2,242,295 | Foard           | ----- | May 20, 1941  |
| 2,369,290 | Foard           | ----- | Feb. 13, 1945 |
| 2,387,984 | Eddy            | ----- | Oct. 30, 1945 |
| 2,445,536 | Parsons et al.  | ----- | July 20, 1948 |
| 2,464,826 | Neher et al.    | ----- | Mar. 22, 1949 |
| 2,516,487 | Schlucksupp     | ----- | July 25, 1950 |
| 2,562,984 | Image           | ----- | Aug. 7, 1951  |
| 2,571,962 | Smith et al.    | ----- | Oct. 16, 1951 |
| 2,583,286 | Albini-Coloinbo | ----- | Jan. 22, 1952 |

#### OTHER REFERENCES

Industrial and Engineering Chem., "Methacrylate Resins," April 1939, pages 382-387.